

## UNITED STATES PATENT OFFICE.

ALAN KISSOCK, OF NEW YORK, N. Y., ASSIGNOR TO CARL M. LOEB, OF NEW YORK, N. Y.

## PROCESS OF MAKING ALLOY STEEL.

No Drawing.

Application filed November 12, 1924. Serial No. 749,561.

To all whom it may concern:

Be it known that I, ALAN KISSOCK, a citizen of the United States, residing at New York, in the county and State of New York, have made certain new and useful Improvements in Processes of Making Alloy Steel, of which the following is a specification.

The invention relates to a novel process of producing alloy steel, and in certain aspects thereof it relates more particularly to a novel process of producing molybdenum alloy steel.

The process consists in the novel steps and process hereinafter described; and the objects and advantages thereof are hereinafter pointed out in part, or will be obvious herefrom or may be ascertained by practicing the invention.

The process is directed primarily to the alloying of steel with a suitable alloying metal while obviating the preliminary reduction of the alloying metal or metallic compound to the metallic state or condition, and also avoiding the addition of slag-forming elements or materials in the reduction of the alloying agent or material in the steel furnace.

It is known in the art to make alloy steel by adding to the fused steel in the furnace the alloying element after it has been reduced to the metallic state, which state in the case of different elements is designated ferro-chromium, ferro-tungsten, ferro-molybdenum, etc.

In the case of molybdenum, it is further known that this metal may be introduced directly into the fused steel as an alloy in the form of certain salts thereof, without the preliminary reduction into the metallic state in the electric furnace already referred to; that is, in the case of molybdenum, without such preliminary reduction to ferro-molybdenum. Two instances of such salts of molybdenum and the direct alloying thereof with the steel are calcium molybdate (as disclosed in my United States Patent No. 1,300,279) and iron molybdate (as disclosed in my United States application Ser. No. 714,769 filed May 21, 1924).

There are many instances, however, in which the use of a salt, or the presence of any chemically combined metal other than the desired alloying element is objectionable and undesirable, as for instance, in the

manufacture of certain high-grade steels. 55 With the attainment of this object primarily in view, in accordance with my present invention, I employ as the alloying agent or substance one of the oxides of molybdenum, preferably the tri-oxide,  $MoO_3$ . 60

These compounds of molybdenum present many advantages for alloying steel. For example, the tri-oxide may be produced directly and simply from high-grade molybdenite ( $MoS_2$ ) concentrates by a simple 65 roasting operation, and without the addition of any diluting material, such for instance as the compounds of iron or calcium. The molybdenum oxide may be introduced into the steel furnace by being added with 70 the charge, or may be introduced into the furnace slag during the regular steel melting process, or at other suitable time, the molybdenum oxide being absorbed into the slag, and the metallic molybdenum 75 being subsequently reduced therefrom by the contact of the molybdenum bearing slag with the molten steel beneath. The metallic molybdenum content of the furnace slag in this manner enters into and alloys with the steel 80 in any desired proportion, dependent upon the amount of molybdenum oxide introduced into the furnace. There is no formation of slag from the decomposition or dissociation of the molybdenum oxide. 85

The process of my present invention is very direct and simple, and is exceedingly economical. It utilizes as the alloying agent a material of higher grade and greater purity, which is more entirely suitable in the 90 manufacture of better steels, as well as being desirable and advantageous in other connections.

It will be understood that the process is likewise workable with other substances 95 which behave in the same general manner chemically and physically and is not limited to the materials herein specifically prescribed, although they constitute the present preferred manner of practicing the invention. 100

What I claim is:—

1. The process of making molybdenum steel comprising adding an oxide of molybdenum directly to the steel furnace during the process of making the steel, whereby the oxide is reduced by the constituents of the steel bath, no other reducing agent being 105

added to effect the reduction of the molybdenum oxide.

2. The process of making molybdenum steel comprising adding a charge consisting solely of substantially pure molybdenum oxide directly to the steel furnace during the process of making the steel, whereby the

oxide is reduced by the steel itself, no other reducing agent being added to effect the reduction of the molybdenum oxide.

In testimony whereof, I have signed my name to this specification.

ALAN KISSOCK.